

F. J. ROOT.  
ART OF TREATING COAL.  
APPLICATION FILED APR. 7, 1919.

1,426,012.

Patented Aug. 15, 1922.



Witnesses:

*W. Taylor,  
A. Kovarik.*

Inventor:  
Frank J. Root,  
*Brydgesworth, Lee, Critten & Miles,  
Atto.*

# UNITED STATES PATENT OFFICE.

FRANK J. ROOT, OF CHICAGO, ILLINOIS.

## ART OF TREATING COAL.

1,426,012.

Specification of Letters Patent. Patented Aug. 15, 1922.

Application filed April 7, 1919. Serial No. 287,957.

*To all whom it may concern:*

Be it known that I, FRANK J. ROOT, a citizen of the United States, residing at Chicago, in the county of Cook and State 5 of Illinois, have invented a new and useful Improvement in the Art of Treating Coal, of which the following is a specification.

This invention relates to improvements 10 in the art of treating coal to obtain therefrom as commercial products the substances derived by the carbonization or thermal decomposition thereof.

In processes involving the application of 15 heat to coal a proper control of the temperature is of great importance, inasmuch as the products obtained vary in character with the temperature conditions prevailing in the treated coal. The character of both the 20 primary and secondary products of decomposition are dependent upon the temperature of treatment, and this may vary in different portions of the coal under treatment in accordance with certain factors, among which 25 the most important are the density and conductivity of the coal, and the uniformity of heating of the mass. Other factors which affect the character more particularly of the secondary products of decomposition, 30 such as the tars, are the length and the thermal characteristics of the passages afforded for the passage of the vapors and gases generated, and their proximity to the heated walls of the retort container. Thus, 35 when a body of coal is placed in a chamber or retort and heat is applied from the exterior the rate at which the interior becomes heated will depend upon the conductivity of the charge, as well as upon the external 40 temperature applied, and the conductivity of the charge will vary largely with its compactness and the proportion of interspaces in the charge. Hence with a low conductivity charge having a high proportion 45 of interspaces, such as those now in use, a high temperature decomposition resulting in a relatively high proportion of cyclic and aromatic compounds will take place in the outer portions of the charge, 50 while within the charge a low temperature decomposition will be effected, a relatively high proportion of aliphatic and naphthalene compounds being formed. It is also apparent that if the retort shape and charge 55 arrangement is such that the vapors formed pass through a relatively cool portion of

the charge (the interior) any secondary decompositions which take place will be largely into aliphatic and naphthalene compounds, whereas if the vapors pass through 60 a more highly heated portion of the charge (the outer layers, for example) a larger proportion of aromatic compounds will be formed in their secondary decomposition. It is hence apparent that a proper control 65 of conditions within the retort with the proper application of heat are necessary for securing economically and efficiently the products desired by the operator in treating the coal.

In accordance with my present invention, 70 I subject the coal to be treated, compacted to a greater or less extent, to the action of heat under conditions such that the primary and secondary decompositions occurring may be controlled in accordance with 75 the products desired. The coal, previously comminuted and, if desired, admixed with a binder, is in my present process compressed into blocks of great compactness 80 and density and of uniform size and may be maintained in their compact state during carbonization or heat application by maintaining pressure upon them during the process. By the use of highly compacted material the conductivity of the material is increased and when subjected to heat, particularly under the conditions hereinafter 85 described, the uniformity of the heat decomposition effected and of the resulting 90 products is greater and their character under more perfect control.

The compacted coal utilized in the practice of this process may be prepared by 95 means of any suitable compressing or briquetting machine, for example, one of the style shown in U. S. Letters Patent No. 980,374, granted to Duryea and White, January 3, 1911. A suitable form for the compacted coal is of blocks or briquets in 100 the form of short cylinders of circular or elliptical cross-section compressed under a pressure of at least three tons per square inch and preferably of eight or ten tons per square inch.

In carrying out the present process, for 105 example, with compacted coal in the form of short cylindrical briquets, the latter are charged into tubular retorts of suitable refractory material in close contact with each other, the retort being of such form as to permit of a considerable contacting surface

with the contained coal and of such size as to provide space for the passage and escape of the vapors and gases formed in the distillation process. Thus for coal briquets 5 having a diameter of 4 to 5 inches and circular in cross section, a tubular retort, having a like cross section of 6 inch diameter, will provide an adequate contact surface and vapor passage. To secure uniformity of 10 heating it is advantageous that the briquets should not exceed 8 to 10 inches in diameter. When arranged in the retort the briquets will form a substantially continuous cylinder against the wall of the retort. To maintain 15 the coal in the compact state during the process of distillation a continuous pressure may be maintained thereupon, for instance, by the use of plungers, the plungers being constantly under the action of weights, 20 springs or hydraulic pressure. Suitable means may be provided for the removal of products of distillation from the retort and for their conveyance into mains and to suitable apparatus for separation into their various 25 constituents. By reason of the compact state of the coal mass it is very rapidly penetrated by the heat and being in cylindrical form it will, in a very short space of time, have a practically uniform temperature 30 throughout. As the coal mass, which is in effect an elongated cylinder, is constantly under applied pressure, a high density of the material is maintained and consequently a high conductivity and a greater uniformity 35 of temperature throughout are likewise maintained. Furthermore, to secure a determined average temperature throughout the body of coal, it is not necessary to apply an external heat as much higher than the 40 desired temperature as is the case in present processes of coal carbonization and distillation. As it appears that there is not so great a difference between the external temperature and the internal temperature of the 45 retort, in the present process the temperature to which the gases and vapors are subjected in their passage through the retort is substantially uniform throughout and not substantially different from that of the coal 50 mass from which they have just generated. A uniform heating effect appears thus to be the result both in the coal mass and in the vapor and gaseous bodies in the retort, both being readily under the control of the operator by a proper regulation of the external 55 heat.

In carrying out my process, I control the temperature applied to the retort in accordance with the character of the product which 60 it is desired to obtain and the character of the coal which is treated. Thus if it is desired to produce what is known as a "smokeless coal" from a bituminous or semi-bituminous material, I apply to the retort an external heat of 400-450° C. The coal bri-

quets acquire a temperature approximating the external temperature of the retort, and this temperature substantially uniform throughout the retort, a removal of the volatile matter of the coal is rapidly effected 70 and without substantial or undue decomposition.

In gas production and by-product coking I may use higher temperatures, the specific temperature utilized varying in accordance 75 with the character of the product desired. In general it may be stated that if it is desired to produce a by-product containing a relatively high proportion of aromatics, temperatures of 1000° C. or above should 80 be used. As is readily apparent, in the present process, it is not necessary that the external temperature applied be as great as that usually applied in gas manufacture and by-product coking, inasmuch as the higher 85 conductivity of the coal mass and the greater uniformity of temperature throughout the retort result in a more rapid penetration of the interior of the coal mass by the heat, a greater uniformity in the products of distillation produced in various parts of the 90 retort and a more adequate control of the character of the products.

In carrying out the present process as applied to the carbonization of coal wherein a 95 temperature of from 400° to 450° C. is applied for the purpose of producing a non-smoking fuel, we may utilize retorts of cast iron or steel, as illustrated in the accompanying drawing, which shows in section apparatus adapted to carry out such an application of the present process.

In the drawing is illustrated in section a furnace 1 of refractory material, provided with suitable heating means, illustrated as 105 a fire grate 2, and with a suitable exit 3 for the waste products of combustion. Within the furnace, and preferably extending therethrough, are a plurality of tubular retorts 4, which may suitably be of circular cross-section. In the utilization of the process for the production of a non-smoking coal, for which temperatures of 400° to 450° C. are required, the retorts may suitably be constructed of cast iron or steel. At one end 110 of the furnace the retorts open into a suitable chamber 5, from which an exit passage 6 is provided to carry away the products resulting from the carbonization of the coal. This chamber is closed from the exterior by 115 means permitting access to the interior of the chamber and the retorts. This is indicated as the door 20 attached to the furnace or to the chamber 5 by suitable hinges 7 and locked for example, by the cam locks 8.

The coal briquets are placed in the retorts 4, the door being open and are so arranged as to form a substantially continuous column or cylinder in the retort. The diameter of the briquets is less than that of the retort, 120

so as to provide a suitable vapor passage between the retort and the briquet. Thus, for a retort of a diameter of approximately 6 inches, the briquets used may have a 5 diameter of  $4\frac{1}{2}$  to 5 inches. The briquets being properly inserted in the retort, means are provided at the charging and discharging end for holding them in position during the process of carbonization. As such means 10 we may provide, for example, plungers 10, of a diameter preferably less than that of the briquets, which enter the retort end and are removably retained in position by any suitable means, such as the screws 11, which 15 pass through the door 20.

In order to exert pressure upon the column of briquets in the retort, or to maintain said column against expansion, I may provide plungers 12, provided with rods 13, 20 which extend through suitable stuffing boxes 14 in the caps 15 of the retorts at the ends opposite their charging and discharging ends. The pressure upon the plungers may be exerted by any desired means, such as 25 weights, springs or hydraulic pressure. In the present embodiment it is applied by means of weights 16, which are attached to the rod 13 by means of cables 17 passing over pulleys 18 mounted on the furnace wall. It 30 is obvious that where it is desired only to prevent expansion of the column of coal briquets in the retort, the plungers 12 may be locked in position and the weights 16 dispensed with. It has been found, however, 35 that advantageous results are secured by maintaining a constant pressure upon the material during the process; for example, with retorts containing briquets  $4\frac{1}{2}$  to 5 inches in diameter, a weight of 100 to 120 40 pounds has been found to produce a well compacted residual coal-like product or non-smoking fuel. With Illinois coal and utilizing a maximum temperature of approximately  $450^{\circ}\text{C}$ ., 77% of the original weight 45 of the fuel was found to remain in the coke-like product in the retort. The column of coal is heated substantially uniformly throughout its length and, by reason of its high conductivity, the thermal conditions 50 are substantially uniform throughout its thickness.

At the termination of the carbonization of the coal, for this purpose, which may take place in from  $2\frac{1}{2}$  to  $3\frac{1}{2}$  hours, the retort may 55 be discharged by opening the doors 20, thereby removing the plungers 10 and forcing the plungers 12 through the retorts to eject the residual material.

In utilizing the process for the production 60 of gas, or for by-product coking, it will be readily apparent to those skilled in the art that retorts of suitable refractory material may be utilized and the temperature and time of treatment controlled in accordance 65 with the character of the decomposition de-

sired. The conditions suitable for the various types of decomposition of the coal have already been set forth in the specification. The volatilized decomposition products will pass off through the passageway between the 70 column of briquets and the retort walls, being subjected to substantially uniform thermal conditions throughout, and will be conducted to suitable separating and purifying devices by pipe 6. 75

Although I have described my invention in connection with certain theories as to the operation thereof, and have also described certain specific embodiments thereof, I do not intend that the scope of my invention shall 80 be limited by the accuracy of the theories set forth, nor to the specific details recited, except in so far as such limitations are included in the accompanying claims. 85

I claim:

1. The process of treating coal by the thermal decomposition thereof, which consists in compacting the coal to a dense block, subjecting the same to the action of heat, applying pressure thereto in one direction, the 90 dense mass being surrounded by a retort of greater size than said body transverse to the direction of application of pressure. 95

2. The process of treating coal by thermal decomposition thereof, which consists in compressing the coal into compact blocks, subjecting a plurality of said blocks, juxtaposed in the form of a column, while surrounded by a retort of greater cross section than said column, to the action of heat. 100

3. The process of treating coal by thermal decomposition thereof, which consists in compacting the coal into dense blocks, subjecting a plurality of said blocks, juxtaposed in the form of a column, while surrounded by a retort of greater cross-section 105 than said column, to the action of heat, and preventing longitudinal expansion of said column. 110

4. The process of treating coal by thermal decomposition thereof, which consists in compacting the coal into dense blocks, subjecting a plurality of said blocks, juxtaposed in the form of a column, while surrounded by a retort of greater cross section 115 than said column, to the action of heat and applying pressure to said column longitudinally thereof. 120

5. The process of treating coal by the thermal decomposition thereof, which consists in compressing coal particles by a pressure of at least three tons per square inch into dense blocks, subjecting said blocks in the form of a continuous column, while surrounded by a retort of greater cross section than said 125 column, to the action of heat applied throughout the length of the column. 130

6. The process of treating coal to produce a smokeless fuel therefrom which consists in compressing coal particles into dense masses 130

by a pressure of at least three tons per square inch and subjecting the dense mass to a temperature of 450° C. uniformly applied throughout.

5. 7. The process of treating coal to produce a smokeless fuel therefrom which consists in compressing coal particles into dense blocks by a pressure of at least three tons per square

inch, applying pressure to said blocks in one direction while subjecting it to a temperature of 450° C., the blocks being surrounded by a retort of larger dimensions transverse to the direction of application of pressure. 10

FRANK J. ROOT.